# EUROPEAN PATENT SPECIFICATION

(11) **EP 0 614 766 B1**
(45) Date of publication and mention of the grant of the patent: **17.09.1997**
(21) Application number: 93301845.9
(22) Date of filing: 11.03.1993
(51) Int. Cl.: B41M 5/00

(54) **Coated paper suitable for ink fusion thermal transfer, and manufacture thereof**
Beschichtetes Papier für die thermische Übertragung von schmelzbaren Tinten und sein Herstellungsverfahren
Papier revêtu utilisable pour le transfert thermique d'encres fusibles et son procédé de fabrication

(43) Date of publication of application: 14.09.1994
(73) Proprietor: Nippon Paper Industries Co Ltd, Tokyo 100 (JP)
(72) Inventor: Yoshida, Yoshio, Sanyo-Kokusaku Pulp Co., Ltd., Shinjuku-ku, Tokyo (JP); Matsukawa, Masao, Sanyo-Kokusaku Pulp Co., Ltd., Chiyoda-Ku, Tokyo (JP); Kuroyama, Yoshihiro, Sanyo-Kokusaku Pulp Co., Ltd., Shinjuku-ku, Tokyo (JP); Shimada, Teruhisa, Sanyo-Kokusaku Pulp Co., Ltd., Shinjuku-ku, Tokyo (JP)
(74) Representative: Dixon, Donald Cossar

(56) References cited:
- EP-A- 0 529 308
- DATABASE WPI,n 90-379954,Derwent Publications Ltd,London,GB; & JP A 2274587 (SANYO) 08-11-1990.

## Description

This invention concerns an ink fusion transfer type of paper, and more specifically, a paper suitable for ink fusion transfer type thermal printers and copiers.

EP 529 308 describes an ink jet recording paper which comprises a support having at least one surface coated with a pigment-containing composition wherein the main pigment component is calcium carbonate compounded silica.

Smooth, high grade recording paper which has been treated by a Super Calendar or the like is used in ink fusion transfer type thermal printers or copiers as it is known to give a clear image. This is particularly true if the recording surface has a smoothness of 100 seconds or more. By making the paper smoother so that there is better contact between the paper and the ink ribbon, more ink is transferred to the paper surface. As a result, reproduction of full tone images is improved, however reproduction of half tone images is unsatisfactory.

At present, coated paper having a high smoothness and gloss is generally not used in ink fusion transfer type thermal printers and copiers. The reason for this is that although the paper is extremely smooth so that there is uniform contact with the ink ribbon, which might be expected to give a good ink copy, transfer of ink actually takes place unevenly and image reproduction is poor.

Non-uniform transfer of ink is particularly evident in the case of smooth, high gloss art paper for printing and in the case of cast-coated paper. This is due to the fact that, as there are very few surface imperfections or cavities, molten ink does not easily stay on the paper and may be retransferred from the paper back to the ink ribbon.

Therefore, although coated paper for printing is designed to be adequate for ordinary printing applications, it is not suitable for ink fusion transfer type thermal printers and copiers.

If these problems inherent in coated printing paper could be resolved, it would be possible to use it for such printers and copiers, and images of higher quality than ever before might be obtained.

In general, in order to confer high surface smoothness on coated paper, the surface is flattened under high pressure using a Super Calendar or similar device. This paper is not as tough as high grade paper, and since it is very dense, it lacks the feeling of volume. In addition, the paper has a low gloss so that there is a very poor balance with the gloss of the image area, and a high image quality comparable to that of ordinary offset printing cannot be obtained.

The inventors, after performing various studies aimed at resolving the aforesaid problems, found that by incorporating a minimum amount of a synthetic silica having a predetermined specific surface in the paper, good results could be achieved with coated paper manufactured by cast coating.

It is therefore an object of this invention to provide a coated paper which not only gives excellent image reproduction when used in ink fusion transfer type thermal printers and copiers, but which also has a high gloss in both the non-image and image parts.

It is a further object of this invention to provide a method of manufacturing a coated paper that can be used in ink fusion transfer type thermal printing applications.

The aforesaid objectives of the invention are attained by an ink fusion transfer paper having a recording layer comprising at least one recording layer on a support, this paper being characterized in that the uppermost layer of the recording layer consists of at least 100 parts by weight of a pigment comprising a synthetic silica together with at least one organic pigment selected from fine particles of styrene resins, acrylic resins and styrene-acrylic copolymer resins and 10 - 50 parts by weight of a binder, the layer being present on one or both sides of the support at a coverage of 5 - 50 g/m² per side in terms of dry solids, 30 - 100 weight percent of the aforesaid pigment consists of a synthetic silica having a specific surface of 20 - 600 m²/g, and the 75 degree gloss of the aforesaid uppermost layer of the paper is no less than 50%.

The synthetic silica used in this invention is generally referred to as non-crystalline silica, amorphous silica, anhydrous silicic acid, hydrated silicic acid, finely powdered silica or white carbon. Its structure is based on a Si-O net, and it is a silicic acid with no fixed crystalline form. From the viewpoint of transferability of molten ink, the synthetic silica used should have a specific surface of 20 - 600 m²/g, and it is particularly preferable that it lies within the range 20 - 300 m²/g. If the specific surface is greater than 600 m²/g or less than 20 m²/g, the reproducibility of half tone images declines although the reason for this is unclear.

The synthetic silica used in this invention may be prepared by the wet method, dry method or aerogel method, there being no particular limitation on the method of preparation.

In this invention, the blending proportion of synthetic silica in the coating solution is 30 - 100 parts by weight with respect to 100 parts of pigment. If this blending proportion is less than 30 parts by weight (i.e. less than 30 weight %), transfer of molten ink to the recording layer is unsatisfactory and reproducibility of half tone images is particularly impaired.

Fine particles of the organic pigments are preferable from the viewpoint of hardness, elasticity and heat resistance. In particular, if fine hollow particles of polystyrene or styrene-methylmethacrylate copolymer are used, it is easier to achieve smoothness of the coated surface and the density of the coated layer can be effectively reduced.

The binder may be a resin, emulsion, latex or natural high polymer which gives a strong adhesion between the pigment and raw paper, and which does not cause blocking between papers or between the paper and ink ribbon, these materials being used either alone or in conjunction with one another.

Examples of such binders are polyvinyl alcohol or starches such as starch oxide, starch esters, enzyme-modified starch and cationic starch, casein, soy proteins, fiber derivatives such as carboxymethyl cellulose and hydroxyethyl cellulose, styrene-acrylic resins, styrene-butadiene resins, vinyl acetate resins and acrylic resins.

The blending proportion of the binder in the coating solution composition is 10 - 50 parts by weight with respect to 100 parts by weight of pigment. If the blending proportion of binder is less than 10 parts by weight, the strength of the coating film declines, and if the proportion is greater than 50 parts by weight, the properties of the coating are adversely affected.

To the coating, dyes or colored pigments may also be added to adjust color, and fluorescent dyes may be added to improve visual whiteness.

The coating containing the aforesaid components may easily be prepared by any of the methods known in the art. Also known additives such as dispersing agents, antifoaming agents, release agents, pH regulating agents, lubricants, water retention agents and preservatives may also be added to the aforesaid coating to the extent that they do not impair the advantage of the invention.

In this invention, the coating solution prepared as described hereintofore is coated on a support to be used as a recording layer. If the surface of paper coated with this solution is simply smoothed by a Super Calendar (Tokkai-sho(nonexamined published Japanese patent application) 62-198876), however, the paper is not tough enough, sufficient paper gloss is not obtained, and it is difficult to transport the paper inside the printer or copier due to the paper's lack of toughness. Further, transferability of ink declines so that a good image is not obtained, and the balance between the gloss of the paper in the image and non-image parts is extremely poor.

If a coated layer is formed by cast coating the aforesaid coating solution on the paper, on the other hand, paper strength is not impaired, extremely high paper gloss is achieved and the thermal transfer paper of this invention is easily obtained, although no definite reasons for this have been given.

The specific surface of the pigment used in paper coatings is generally 2 - 3 g/m² and no greater than 10 m²/g. On the other hand, the specific surface of the synthetic silica used in this invention is 20 - 600 m²/g. This is far greater than that of pigments commonly used, and it leads to the following inferences.

In a coated layer produced by cast coating, the synthetic silica of high specific surface is incorporated in the recording layer without undergoing any modification which thus gives rise to a very large number of cavities. It may be conjectured that this results in better transferability of ink, absorption of molten ink by the cavities so that image surface imperfections are reduced, and reduction of surface scattering reflections so that image gloss is heightened.

A single or multiple coating is applied by either an on-line or an off-line coater to one or both sides of the paper such that the dry weight of coating on each side is 5 - 50 g/m², and preferably 8 - 30 g/m². If the amount of coating is less than 5 g/m², the film on the surface of the raw paper is insufficient so that a high paper gloss cannot be obtained, while if it is greater than 50 g/m², the paper density increases so that it becomes less tough, paper transport is problematic and the paper loses its function as a printing and copying paper.

The cast coating method used may be any suitable method known in the art such as solidification, rewetting or wetting, providing using a casting drum having a mirror surface.

There is no particular limitation on the coating technique employed to obtain the recording layer, it being possible to use any ordinary coating technique such as blade coating, roller coating, air knife coating and bar coating.

The solidifying agent used in cast coating by solidification is commonly formic acid, acetic acid, succinic acid, tartaric acid, lactic acid, hydrochloric acid, calcium, zinc, barium, lead, magnesium, cadmium or aluminum sulfates, potassium sulfate, potassium succinate, borax or boric acid, however this invention is not limited to only these substances. Further, the choice of a suitable binder which solidifies well together with these solidifying agents is effective in improving coating speed and the finish of the coated surface.

The raw paper may be an acid or neutral high or medium grade paper. For coating purposes, however, it is preferable that the paper be prepared by known methods of raw paper blending, preparation and manufacture (Tokkai Sho 55-47385).

As described hereintofore, the ink fusion transfer paper of this invention has an extremely high gloss, allows good ink transfer and gives an excellent image gloss. It therefore offers a good paper/image gloss balance, a high quality image, and is particularly suitable as a paper for ink fusion transfer type thermal printers and copiers.

### EXAMPLES

This invention will now be described in more detail by means of the following examples, but it is to be understood that it is not limited by them in any way. All parts given in the examples are parts by weight.

The measurements in the examples were performed as follows:
(1) Density: Measured according to the method of JIS P8118.
(2) Smoothness: Measured according to the method of JIS P8119.
(3) Gloss: The 75° gloss of the coated surface was measured according to the method of JIS P8142.
(4) Image gloss: Patterns having a half tone dot surface proportion of 25%, 50% and 100% respectively were recorded using a Mitsubishi Color Thermal Printer M4234-10, and the gloss of each pattern was measured.
(5) Image reproducibility test: Ink transfer performance in the 25% half tone dot pattern was judged visually.
   If the pattern was uniformly recorded, it was graded by "○", if some parts were missing it was graded by "△", and if practically no ink had been transferred it was graded by "X".
(6) Coating strength: Using an IGT Print Suitability Tester (IGT A-1type machine manufactured by IGT K.K.), an ink tack of 10, ink volume of 0.025 cc and print speed of 1.2 m/sec, patterns where none of the ink that had been transferred came off were graded by "○", patterns where some of the ink came off were graded by "△" and patterns where all the ink came off were graded by "X".

### EXAMPLE 1

10 parts heavy calcium carbonate, 1 part cationic starch and 0.1 parts of a sizing agent (alkyl ketene dimer) were blended with 100 parts of a bleached broadleaf tree kraftpulp slurry of beating degree 400 cc (L-BKP) so as to make a raw paper of weighting 69 g/m².

A coating solution containing 55% dry solids was also prepared from 30 parts synthetic silica (commercial name: Syloid 404, Fuji Davison K.K., specific surface 300 m²/g) 40 parts primary grade kaolin (commercial name: Ultrawhite 90, E.M.C. K.K.) and 20 parts calcium carbonate (commercial name: Brilliant 15, Shiraishi K.K.) as pigments together with 10 parts of an organic pigment (commercial name: Boncoat PP-1100, Dai Nippon Kagaku K.K.), 15 parts styrene butadiene latex and 15 parts casein as binders, and 2 parts calcium stearate as a release agent.

The coating solution obtained was applied to the aforesaid raw paper by means of a roll coater as in Comparative Example 1, excepting that the rate of application was 40 g/m² in terms of dry solids. An ink fusion transfer thermal paper of weighting 109 g/m² was thus obtained.

### COMPARATIVE EXAMPLE 1

10 parts heavy calcium carbonate, 1 part cationic starch and 0.1 parts of a sizing agent (alkyl ketene dimer) were blended with 100 parts of a bleached broadleaf tree kraftpulp slurry of beating degree 400 cc (L-BKP) so as to make a raw paper of weighting 92 g/m².

A coating solution containing 43% dry solids was also prepared from 80 parts synthetic silica (commercial name: Syloid 404, Fuji Davison K.K., specific surface 300 m²/g) and 20 parts primary grade kaolin (commercial name: Ultrawhite 90, E.M.C. K.K.) as pigments, 5 parts styrene butadiene latex and 5 parts casein as binders, and 2 parts calcium stearate as a release agent.

After applying the coating solution obtained to the aforesaid raw paper by means of a roll coater at a rate of 10 g/m² in terms of dry solids, the coating was solidified using a 10% aqueous solution of zinc formate as solidifying agent, and while the coating film was still wet, it was dried in pressure contact with a casting drum having a mirror surface heated to 100°C. An ink fusion transfer thermal paper of weighting 102 g/m² was thus obtained.

### COMPARATIVE EXAMPLE 2

A coating solution containing 42% dry solids was prepared from 80 parts synthetic silica (commercial name: Syloid 404, Fuji Davison K.K., specific surface 300 m²/g) and 20 parts primary grade kaolin (commercial name: Ultrawhite 90, manufactured by E.M.C. K.K.) as pigments, 15 parts styrene butadiene latex and 15 parts casein as binders, and 2 parts calcium stearate as a release agent.

The coating solution obtained was applied to the raw paper of Comparative Example 1 (92 g/m²) by means of a roll coater in the same manner as that of Comparative Example 1, excepting that the application rate was 15 g/m² in terms of dry solids. An ink fusion transfer thermal paper of weighting 107 g/m² was thus obtained.

### COMPARATIVE EXAMPLE 3

A coating solution containing 46% dry solids was prepared from 100 parts synthetic silica (commercial name: Mizukasil P-527, Mizusawa Industrial Chemicals K.K., specific surface 30 m²/g) as a pigment, 20 parts styrene butadiene latex and 20 parts casein as binders, and 2 parts calcium stearate as a release agent.

The coating solution obtained was applied to the raw paper of Comparative Example 1 by means of a roll coater such that the application rate was 10 g/m² in terms of dry solids in the same manner as that of Comparative Example 1. An ink fusion transfer thermal paper of weighting 102 g/m² was thus obtained.

### COMPARATIVE EXAMPLE 4

The synthetic silica used in Comparative Example 3 was replaced by a pigment having a specific surface of 600 m²/g (commercial name: Syloid 600, Fuji Davison K.K.), 23 parts styrene butadiene latex and 20 parts casein added as binders, then 2 parts calcium stearate added as a release agent so as to obtain a coating solution containing 40% solids. The coating solution obtained was applied to the raw paper of Comparative Example 1 by means of a roll coater in the same manner as that of Comparative Example 1 excepting that the application rate was 5 g/m² in terms of dry solids.

An ink fusion transfer thermal paper of weighting 97 g/m² was thus obtained.

### COMPARATIVE EXAMPLE 5

A coating solution containing 54% dry solids was prepared from 30 parts synthetic silica (commercial name: Syloid 404, Fuji Davison K.K., specific surface 300 m²/g), 40 parts primary grade kaolin (commercial name: Ultrawhite 90, E.M.C. K.K.) and 30 parts calcium carbonate (commercial name: Brilliant 15, Shiraishi K.K.) as pigments, 15 parts styrene butadiene latex and 10 parts casein as binders, and 2 parts calcium stearate as a release agent.

The coating solution obtained was applied to the raw paper of Comparative Example 1 (92 g/m²) by means of a roll coater in the same manner as that of Comparative Example 1, excepting that the application rate was 12 g/m² in terms of dry solids. An ink fusion transfer thermal paper of weighting 104 g/m² was thus obtained.

### COMPARATIVE EXAMPLE 6

A coating solution containing 58% dry solids was prepared from 5 parts synthetic silica (commercial name: Syloid 404, Fuji Davison K.K., specific surface 300 m²/g), 40 parts primary grade kaolin (commercial name: Ultrawhite 90, E.M.C. K.K.) and 55 parts calcium carbonate (commercial name: Brilliant 15, Shiraishi K.K.) as pigments, 15 parts styrene butadiene latex and 10 parts casein as binders, and 2 parts calcium stearate as a release agent.

This coating solution was applied to the raw paper of Comparative Example 1 by means of a roll coater exactly as in Comparative Example 1, excepting that the rate of application was 15 g/m² in terms of dry solids. An ink fusion transfer thermal paper of weighting 107 g/m² was thus obtained.

### COMPARATIVE EXAMPLE 7

A coating solution containing 58% dry solids was prepared from 25 parts synthetic silica (commercial name: Syloid 404, Fuji Davison K.K., specific surface 300 m²/g), 40 parts primary grade kaolin (commercial name: Ultrawhite 90, E.M.C. K.K.) and 35 parts calcium carbonate (commercial name: Brilliant 15, Shiraishi K.K.) as pigments, 15 parts styrene butadiene latex and 15 parts casein as binders, and 2 parts calcium stearate as a release agent.

This coating solution was applied to the raw paper of Comparative Example 1 by means of a roll coater exactly as in Comparative Example 1, excepting that the rate of application was 15 g/m² in terms of dry solids. An ink fusion transfer thermal paper of weighting 107 g/m² was thus obtained.

### COMPARATIVE EXAMPLE 8

A coating solution was applied to a raw paper by means of a roll coater exactly as in Comparative Example 1, excepting that the application rate was 60 g/m² in terms of dry solids. An ink fusion transfer thermal paper of weighting 129 g/m² was thus obtained.

### COMPARATIVE EXAMPLE 9

A coating solution containing 60% dry solids was prepared from 30 parts synthetic silica (commercial name: FK 700, Degusa K.K., specific surface 700 m²/g), 40 parts primary grade kaolin (commercial name: Ultrawhite 90, E.M.C. K.K.) and 30 parts calcium carbonate (commercial name: Brilliant 15, Shiraishi K.K.) as pigments, 11 parts styrene butadiene latex and 11 parts casein as binders, and 2 parts calcium stearate as a release agent.

This coating solution was applied to the raw paper of Comparative Example 1 by means of a roll coater exactly as in Comparative Example 1, excepting that the rate of application was 11 g/m² in terms of dry solids. An ink fusion transfer thermal paper of weighting 103 g/m² was thus obtained.

### COMPARATIVE EXAMPLE 10

A coating solution containing 56% dry solids was prepared from 30 parts synthetic silica (commercial name: Syloid 404, Fuji Davison K.K., specific surface 300 m²/g) and 70 parts calcium carbonate (commercial name: Brilliant 15, Shiraishi K.K.) as pigments, and 22 parts styrene butadiene latex and 2 parts starch oxide as binders.

This coating solution was applied to the raw paper of Comparative Example 1 by means of a roll coater such that the rate of application was 10 g/m², and dried to give a coated paper of weighting 102 g/m². The coated surface was then smoothed by means of a Super Calendar so as to obtain an ink fusion transfer thermal paper.

Coating solution compositions, specific surfaces of synthetic silica and coating amounts used for each of the ink fusion transfer thermal papers in the aforesaid Example and Comparative Examples are summarized in Table 1. In this Table, the figures in the pigment column represent the ratios synthetic silica/kaolin/calcium carbonate/organic pigment, and the figure in the binder column represents the ratio latex/casein.

**Table 1**

| Coating Solution | | | Specific Surface of Synthetic Silica (m²/g) | Application Rate (g/m²) |
|---|---|---|---|---|
| | Pigment | Binder | | |
| Example 1 | 30/40/ 20/10 | 15/ 15 | 300 | 40 |

| Comparative Example | | | | |
|---|---|---|---|---|
| 1 | 80/20/ 0/ 0 | 5/ 5 | 300 | 10 |
| 2 | 80/20/ 0/ 0 | 15/ 15 | 300 | 15 |
| 3 | 100/ 0/ 0/ 0 | 20/ 20 | 30 | 10 |
| 4 | 100/ 0/ 0/ 0 | 23/ 20 | 600 | 5 |
| 5 | 30/40/ 30/ 0 | 15/ 10 | 300 | 12 |
| 6 | 5/40/ 55/ 0 | 15/ 10 | 300 | 15 |
| 7 | 25/40/ 35/ 0 | 15/ 15 | 300 | 15 |
| 8 | 30/40/ 20/10 | 15/ 15 | 300 | 60 |
| 9 | 30/40/ 30/ 0 | 11/ 11 | 700 | 11 |
| 10 | 30/ 0/ 70/ 0 | 22/ 0 | 300 | 10 |

Paper quality test results and image quality test results for the coated papers obtained as described hereinbefore are given in Table 2.

The results shown in Table 2 confirm not only that the ink fusion transfer thermal paper of this invention has a high paper gloss, is tough and of extremely high quality, but also that images recorded on this paper have a high gloss and that the quality of these images is excellent.

**Table 2**

| | Density (g/cm³) | Smoothness (second) | Gloss Degree (%) 19 | Image Gloss (%) | | | Image Reproducibility | Strength of Coating Layer |
|---|---|---|---|---|---|---|---|---|
| | | | | Half Tone Dot Surface Proportion (%) | | | | |
| | | | | 25 | 50 | 100 | | |
| Example 1 | 0.87 | 1900 | 71 | 83 | 85 | 94 | ○ | ○ |

| Comparative Example | | | | | | | | |
|---|---|---|---|---|---|---|---|---|
| 1 | 0.89 | 500 | 60 | 70 | 81 | 92 | ○ | ○ |
| 2 | 0.90 | 520 | 62 | 72 | 81 | 91 | ○ | ○ |
| 3 | 0.91 | 630 | 55 | 65 | 74 | 93 | ○ | ○ |
| 4 | 0.89 | 550 | 53 | 63 | 73 | 91 | ○ | ○ |
| 5 | 0.91 | 2500 | 73 | 83 | 88 | 92 | ○ | ○ |
| 6 | 0.91 | 3900 | 85 | 85 | 86 | 88 | X | ○ |
| 7 | 0.90 | 2200 | 75 | 75 | 86 | 88 | △ | ○ |
| 8 | 0.98 | 2300 | 78 | 76 | 85 | 80 | ○ | △ |
| 9 | 0.91 | 2600 | 54 | 54 | 60 | 75 | △ | ○ |
| 10 | 1.29 | 1200 | 28 | 33 | 56 | 66 | X | ○ |

## Claims

1. An ink fusion transfer paper comprising at least one recording layer on a support, the paper being characterized in that the uppermost layer of the recording layer consists of at least 100 parts by weight of a pigment comprising a synthetic silica together with at least one organic pigment selected from fine particles of styrene resins, acrylic resins and styrene-acrylic copolymer resins and 10-50 parts by weight of a binder, the layer being present on one or both sides of the support at a coverage of 5-50 g/m² per side in terms of dry solids, 30-100 weight percent of the aforesaid pigment consists of a synthetic silica having a specific surface of 20-600m ²/g, and the 75 degree gloss of said uppermost layer is no less than 50%.

2. An ink fusion transfer paper as claimed in Claim 1, wherein said organic pigment is fine hollow particles of polystyrene or a styrene-methylmethacrylate copolymer.

3. An ink fusion transfer paper as claimed in Claim 1 or 2, wherein the binding agent is selected from a polyvinyl alcohol, starches, casein, soy protein, fiber derivatives, styrene-acrylic resins, styrene-butadiene resins, vinyl acetate resins and acrylic resins.

4. An ink fusion transfer paper as claimed in Claim 3, wherein the starches consist of a starch oxide, a starch ester, an enzyme-modified starch or a cationic starch and the fiber derivatives consist of a carboxymethyl cellulose or hydroxyethyl cellulose.

5. An ink fusion transfer paper as claimed in any preceding claim, wherein at least one dye which can be a fluorescent dye and/or colored pigment is also contained in the uppermost layer.

6. An ink fusion transfer paper as claimed in any preceding claim, wherein the uppermost layer is present on one or both sides of the support at a coverage of 8-30 g/m² per side in terms of dry solids.

7. A method of manufacturing an ink fusion transfer paper as claimed in any preceding claim, characterized in that the uppermost layer is prepared by a cast coating method.

8. A method as claimed in Claim 7, wherein the cast coating is carried out by a solidification method.

9. A method as claimed in Claim 8, wherein at least one solidifying agent selected from formic acid, acetic acid, succinic acid, tartaric acid, lactic acid, hydrochloric acid, a sulfate of calcium, zinc, barium, lead, magnesium, cadmium, aluminum or potassium, potassium succinate, borax or boric acid is contained in a coating solution for said layer.

## Patentansprüche

1. Papier für die Schmelzübertragung von Tinte, das mindestens eine Aufzeichnungsschicht auf einem Träger umfaßt, wobei das Papier dadurch gekennzeichnet ist, daß die oberste Schicht der Aufzeichnungsschicht aus mindestens 100 Gewichtsteilen Pigment, das synthetisches Siliciumdioxid zusammen mit mindestens einem organischen Pigment ausgewählt aus feinen Teilchen aus Styrolharzen, Acrylharzen und Styrol/Acryl-Copolymerharzen umfaßt, und 10 bis 50 Gewichtsteilen Bindemittel besteht, wobei die Schicht auf einer oder beiden Seiten des Trägers mit einer Bedeckung von 5 bis 50 g/m² pro Seite, im Bezug auf trochene Feststoffe, vorhanden ist, wobei 30 bis 100 Gew.-% des zuvor genannten Pigments aus synthetischem Siliciumdioxid mit einer spezifischen Oberfläche von 20 bis 600 m²/g bestehen und der 75° Glanz der obersten Schicht nicht kleiner 50 % ist.

2. Papier für die Schmelzübertragung von Tinte nach Anspruch 1, bei dem das organische Pigment aus feinen Hohlteilchen aus Polystyrol oder einem Styrol/Methylmethacrylat-Copolymer besteht.

3. Papier für die Schmelzübertragung von Tinte nach Anspruch 1 oder 2, bei dem das Bindemittel ausgewählt ist aus Polyvinylalkohol, Stärken, Casein, Sojaprotein, Faserderivaten, Styrol/Acryl-Harzen, Styrol/Butadien-Harzen, Vinylacetatharzen und Acrylharzen.

4. Papier für die Schmelzübertragung von Tinte nach Anspruch 3, bei dem die Stärken aus Stärkeoxid, Stärkeester, enzym-modifizierter Stärke oder kationischer Stärke bestehen und die Faserderivate aus Carboxymethylcellulose oder Hydroxyethylcellulose bestehen.

5. Papier für die Schmelzübertragung von Tinte nach einem der vorhergehenden Ansprüche, bei dem in der obersten Schicht außerdem mindestens ein Farbstoff enthalten ist, der ein Fluoreszenzfarbstoff und/oder gefärbtes Pigment sein kann.

6. Papier für die Schmelzübertragung von Tinte nach einem der vorhergehenden Ansprüche, bei dem die oberste Schicht auf einer oder beiden Seiten des Trägers mit einer Bedeckung von 8 bis 30 g/m² pro Seite, in Bezug auf trockene Feststoffe, vorhanden ist.

7. Verfahren zur Herstellung eines Papiers für die Schmelzübertragung von Tinte gemäß einem der vorhergehenden Ansprüche, dadurch gekennzeichnet, daß die oberste Schicht durch ein Gießbeschichtungsverfahren hergestellt wird.

8. Verfahren nach Anspruch 7, bei dem die Gießbeschichtung durch ein Verfestigungsverfahren ausgeführt wird.

9. Verfahren nach Anspruch 8, bei dem mindestens ein Verfestigungsmittel ausgewählt aus Ameisensäure, Essigsäure, Bernsteinsäure, Weinsäure, Milchsäure, Salzsäure, einem Sulfat von Calcium, Zink, Barium, Blei, Magnesium, Cadmium, Aluminium oder Kalium, Kaliumsuccinat, Borax oder Borsäure in einer Beschichtungslösung für diese Schicht enthalten ist.

## Revendications

1. Papier de transfert d'encre par fusion comprenant au moins une couche d'enregistrement sur un support, le papier étant caractérisé en ce que la couche supérieure de la couche d'enregistrement comprend au moins 100 parties en poids d'un pigment comprenant une silice synthétique avec au moins un pigment organique choisi parmi de fines particules de résines styrène, de résines acryliques et de résines copolymères styrène-acrylique et 10-50 parties en poids d'un liant, la couche étant présente sur un côté ou sur les deux côtés du support à un taux d'application de 5-50 g/m² par côté en termes de solides secs, 30-100 % en poids du pigment précité consistant en une silice synthétique ayant une surface spécifique de 20-600 m²/g, et le brillant à 75 degrés de ladite couche supérieure n'étant pas inférieur à 50 %.

2. Papier de transfert d'encre par fusion selon la revendication 1, dans lequel ledit pigment organique est constitué par de fines particules creuses de polystyrène ou d'un copolymère de styrène et de méthacrylate de méthyle.

3. Papier de transfert d'encre par fusion selon la revendication 1 ou la revendication 2, dans lequel l'agent de liaison est choisi parmi les suivants : alcool de polyvinyle, amidons, caséine, protéine de soja, dérivés de fibres, résines styrène-acryliques, résines styrène-butadiène, résines acétate de vinyle et résines acryliques.

4. Papier de transfert d'encre par fusion selon la revendication 3, dans lequel les amidons comprennent un oxyde d'amidon, un ester d'amidon, un amidon modifié par des enzymes ou un amidon cationique, et les dérivés de fibres comprennent une carboxyméthylcellulose ou une hydroxyéthylcellulose.

5. Papier de transfert d'encre par fusion selon l'une des revendications précédentes, dans lequel au moins un colorant, qui peut être un colorant fluorescent et/ou un pigment coloré, est également contenu dans la couche supérieure.

6. Papier de transfert d'encre par fusion selon l'une des revendications précédentes, dans lequel la couche supérieure est présente sur un côté ou sur les deux côtés du support à un taux d'application de 8-30 g/m² par côté en termes de solides secs.

7. Procédé de fabrication d'un papier de transfert d'encre par fusion selon l'une des revendications précédentes, caractérisé en ce que la couche supérieure est préparée par un procédé de couchage par moulage.

8. Procédé selon la revendication 7, dans lequel le couchage par moulage est effectué par un procédé de solidification.

9. Procédé selon la revendication 8, dans lequel au moins un agent de solidification sélectionné parmi les suivants : acide formique, acide acétique, acide succinique, acide tartarique, acide lactique, acide chlorhydrique, sulfate de calcium, de zinc, de baryum, de plomb, de magnésium, de cadmium, d'aluminium ou de potassium, succinate de potassium, borax ou acide borique, est contenu dans une solution d'enduction pour ladite couche.
